

Aug. 6, 1935.

J. J. STONE

2,010,650

PROCESS FOR PRODUCING ARMOR PLATES

Filed Sept. 3, 1931

2 Sheets-Sheet 1



*Fig. 1.*



*Fig. 2.*



*Fig. 3.*



*Fig. 4.*

Inventor

*John J. Stone.*

By *R. S. C. Dougherty.*  
Attorney

Aug. 6, 1935.

J. J. STONE

2,010,650

PROCESS FOR PRODUCING ARMOR PLATES

Filed Sept. 3, 1931

2 Sheets-Sheet 2

*Fig. 5.*



*Fig. 6.*



*Fig. 7.*



*Fig. 8.*



*Fig. 9.*



Inventor

*John J. Stone.*

By *R. S. C. Keougherty*  
Attorney

## UNITED STATES PATENT OFFICE

2,010,650

## PROCESS FOR PRODUCING ARMOR PLATES

John J. Stone, Bethlehem, Pa., assignor to Bethlehem Steel Company, a corporation of Pennsylvania

Application September 3, 1931, Serial No. 560,929

2 Claims. (Cl. 29—160.4)

My invention relates to an improved process for the manufacture of wrought steel articles and more particularly of forged plates such as armor plates.

5 The object of my invention is to eliminate in large measure from the wrought article the portion of the ingot which is adversely affected by segregation, and to obtain improved physical properties throughout the metal. To this end I 10 use a corrugated ingot and forge two plates therefrom—the major portion of each plate being taken from the external zones of the ingot.

As is well known in the art, a selective freezing action takes place during the solidification of 15 an ingot whereby the metal which solidifies first near the ingot surface contains more iron and less of the minor constituents of the steel (carbon, manganese, phosphorus, sulphur, etc.) than the average composition of the liquid metal. As 20 freezing progresses toward the center of the ingot, the proportion of minor constituents increases until there is produced a marked zone of "segregation" at the core. This central core is also apt to contain voids due to shrinkage of the 25 surrounding metal unless skill is used in so designing the ingot and controlling the pouring process that the voids are filled by molten metal fed from the top. Since solidification proceeds from the bottom of the ingot as well as from the 30 sides, there is a tendency for the upper portion of the core to be most seriously affected by segregation and, in spite of the best ingot design and pouring practice, there is always a conical shaped 35 zone at the top of the core containing porous metal and known as the "pipe". In order to completely remove the "pipe" it is common practice to discard from the top of a large ingot as much as 30% or more of the ingot weight.

The approximate location and shape of the 40 "pipe" in various ingots—together with the consecutive steps in my improved forging process—are illustrated in the drawings which form part of this specification.

Fig. 1 represents an "armor plate ingot";

45 Fig. 2 shows the ingot of Fig. 1 in longitudinal section;

Fig. 3 shows a corrugated ingot such as used in my improved process for making armor plate;

50 Fig. 4 is a longitudinal section of the ingot of Fig. 3; and

Figs. 5, 6, 7, 8, and 9 illustrate successive stages in the forging of the ingot of Fig. 3 by my process.

In producing flat forgings such as armor plate rectangular ingots have been almost universally used heretofore. In fact a particular type of

rectangular ingot has come to be known as an "armor plate ingot". The characteristic proportions of this ingot are a height or length approximately equal to its width, and a thickness equal to one fourth or one fifth of same. The corners 5 are only slightly rounded. The advantages of this type of ingot for producing armor plate reside in the relative ease with which it may be handled under the forging press and in the fact that the segregated core is spread out fairly uniformly 10 over a considerable portion of the width of the ingot. The general shape of an ingot of this type and the location and extent of the pipe and zone of segregation therein are illustrated in Figs. 1 and 2. While the presence of the segregated zone 15 is undesirable it has been found less deleterious to have it spread out in this way than to have it concentrated along a definite line in the finished plate—as would be the case for example if a square ingot were used.

Two major disadvantages of the armor plate 20 type of ingot are its tendency to form surface cracks in cooling or subsequent forging and the practical impossibility of removing segregated metal from the body of the ingot. A further disadvantage inherent in the process of making plate 25 from rectangular ingots is the fact that a large part of the mechanical work of forging only produces elongation of the ingot crystals parallel to the long dimension of the finished plate. The result is that the physical properties of the plate as 30 determined on transverse specimens are markedly inferior to those on longitudinal specimens. While this is true of many steel products—particularly rolled sections—and is taken into account in designing, it is obviously undesirable.

It has long been recognized that corrugated ingots are less apt to develop cracks in cooling and forging than rectangular ingots due to the more 40 favorable arrangement of crystals adjacent their surfaces. Fig. 3 illustrates an ingot of this type and Fig. 4 which is a longitudinal section of the ingot of Fig. 3 shows the location of the segregated zone therein. Figures 5, 6, 7, 8, and 9 illustrate successive stages in my improved forging 45 process as applied to plates. Fig. 5 shows the ingot of Fig. 3 after being rounded up and after the removal of discard metal from both ends. In Fig. 6 the cylindrical faggot of Fig. 5 has been spread and edged to a rectangular shape. Fig. 7 50 shows its condition after further transverse forging. In Fig. 8 the slab has been cut in two parallel to the axis of the ingot. Fig. 9 shows the plates forged longitudinally to finished dimensions plus trimming allowance.

5

10

15

20

25

30

35

40

45

50

55

It is obvious that the transverse forging illustrated by Figs. 6 and 7, followed by the longitudinal forging shown in Figs. 8 and 9 has a tendency to equalize the mechanical work applied to the ingot structure in these directions and that the physical properties of the resulting plate will be more nearly uniform with respect to the directions in which they are determined. The most important feature of my process, however, is the forging of two plates from a single ingot—the parting cut being made through the axis of the ingot. If it were otherwise desirable to forge a single plate from a corrugated ingot the presence of a concentrated zone of segregated metal along the longitudinal axis of the plate would make the product undesirable; but by making the plates from metal which is largely outside this zone and by eliminating the major portion thereof in the trimming allowance between plates I obtain the advantages of great reduction in cross section and of forging in two directions without the detrimental effect of concentrated segregation.

I have heretofore referred to the production of two plates from a single ingot but it will be readily understood that any even number of plates may be produced from an ingot without losing the advantages set forth. In the manufacture of armor plate it is convenient to produce plates in pairs since two identical plates of each size and shape are ordinarily required for a ship—one starboard and one port. It is my preferred practice to cast a corrugated ingot of sufficient size to produce two large plates or four small ones. As a matter of convenience, I prefer to cut the cross forged slab longitudinally while hot. When the forging operations on the individual slabs are completed the finished dimensions of the

plate are then laid out on the slab so that the maximum trimming allowance is on the side adjacent the parting cut. This permits removing the major portion of the segregated zone when the plates are machined to finished size. However, it may be desirable in certain cases to cut a strip either hot or cold from the center of the cross forged slab in order to more completely remove the segregated zone. The heavy sections and the variety of sizes and shapes of armor plates ordinarily preclude rolling as a manufacturing process. Since I have confined this illustration of my process to armor plate, I have consistently referred to forging as the method of working or shaping the metal. The advantages of my process however, may also be secured in the manufacture of lighter and more uniform steel articles by rolling. These variations in procedure come within the scope of my invention.

Having thus described my invention what I claim as new and desire to secure by Letters Patent is:

1. In the production of armor plate the steps of forging a corrugated ingot of substantially circular cross section transversely to its major axis, severing the resulting slab through said axis and forging the resulting portions parallel to said axis.
2. In the production of armor plate the steps of forging a corrugated ingot of substantially circular cross section transversely to its major axis, severing the resulting slab through said axis, forging the resulting portions parallel to said axis, and removing a portion of the metal from the edges of said portions adjacent the parting cut.

JOHN J. STONE.